

# UNITED STATES PATENT OFFICE.

WILHELM A. KOHNCKE, OF LEWISTOWN, ILLINOIS.

## COMPOSITION FOR MAKING WATERPROOF AND FIREPROOF ROOFS, &c.

1,264,307.

Specification of Letters Patent. Patented Apr. 30, 1918.

No Drawing.

Application filed December 20, 1916. Serial No. 137,973.

*To all whom it may concern:*

Be it known that I, WILHELM A. KOHNCKE, a citizen of the United States, and a resident of the city of Lewistown, county of 5 Fulton, and State of Illinois, have invented certain new and useful Improvements in Composition for Making Waterproof and Fireproof Roofs, &c., of which the following is a specification.

10 This invention relates broadly to a mixture of ingredients to form a composition of matter more particularly adaptable for use in making water proof and fire proof roofs and the like.

15 The principal object of this invention is to provide a composition of matter which will be sufficiently plastic when mixed to be laid in suitable layers to constitute a protective covering such as a roof, and wherein 20 the material possesses great adhesive abilities to enable the material to be securely and easily attached to other building materials whereby gutters, flashings, etc., may be omitted when this material is used for forming a roof or the like.

25 A still further object of the present invention is to provide a composition of matter wherein the finished article possesses the required amount of elasticity and at the same time provides an extremely hard wearing surface and is of great strength for a 30 unit cross-sectional area enabling the material to be used in relatively thin layers to accomplish satisfactory results in providing for suitable roofs and the like.

35 A still further object of the present invention is to provide a mixture of materials capable of being transported in the dry state and subsequently mixed with suitable liquids 40 to constitute a composition of matter adaptable for roofing and similar purposes, and possessing water proof and fire proof characteristics and at the same time capable of manipulation when mixed, in either a warm 45 or cold atmosphere.

50 A still further object of the present invention is to provide a suitable composition of matter composed of fire proofing and water proofing ingredients and adapted to be transported in substantially the form of a dry mixture which when mixed with a suitable liquid forms a roof or similar structure of great strength and hardness.

55 Further and other objects of the present invention will in part be obvious and will

in part be pointed out hereinafter in the specification following.

Various types of plastic roofing materials have been heretofore devised and particularly concrete or asphaltic compounds. The 60 concrete structures are objectionable in that the amount of weight required is excessive and also in view of the difficulty in providing for suitable water proofing of the concrete whereby moisture is prevented from 65 entering the pores. Since any freezing in the concrete will sooner or later destroy the roofing structure, asphaltic and gravel roofs are objectionable, first, in the matter of weight and secondly, in the matter of 70 upkeep in that the materials being partially soluble, particularly in rain water the natural elements tend to gradually destroy the structures and the cleaning of snow, etc., from the roof tends to remove a portion 75 of the roofing material itself.

The composition which will hereinafter be more particularly set forth comprises a mixture of materials which sets into a body of great hardness and strength and which 80 body is substantially unaffected by freezing, and is of itself water proof and non-soluble in rain water. The result of this is that a roof or similar structure formed of the composition hereinafter to be described may be 85 of relatively light weight and at the same time will possess a relatively smooth surface of great hardness so that the roof may be easily cleaned and where the same is laid upon an inclined roofing frame there is no 90 tendency whatever of the material to run or move upon itself as is the tendency of all asphaltic or pitch roofs.

The present invention relates more particularly to the materials which are to be 95 used in securing the desiderata above set forth, and comprise a mixture including calcined magnesite, asbestos, sawdust oiled with China wood oil, crushed quartz, talc, marble flour, and carborundum fire sand, or 100 similar material of this character. These ingredients are adapted to be treated by a suitable liquid such as a binder comprising magnesium chlorid dissolved in water.

In disclosing the ingredients and proportions of my invention, the proportions hereinafter referred to are set forth in measure by bulk instead of weight, or in other words in dry measure.

In preparing the ingredients or materials 110

entering into my compound I use sawdust, preferably hard wood sawdust, and prepare two grades of fineness of this sawdust by first sifting a portion of the sawdust through 5 a screen of twenty (20) mesh fineness to the inch and then sifting another portion of sawdust through a screen of fineness of fifty (50) meshes to the inch. After these two 10 grades of sawdust have been obtained they are preferably treated separately with an oily substance known in the art as China wood oil in the proportion of one part by measure of oil to twenty (20) parts of sawdust. The oil and sawdust may be mixed in 15 any suitable manner and in order to insure a thorough mixing, the sawdust is again passed through suitable screens, for example the sawdust that has been passed through the twenty (20) mesh screen is again 20 passed through this screen after the sawdust has been oiled and the sawdust which has passed through the fifty (50) mesh screen is, after being oiled, again passed through this same screen. This second manipulation 25 through the screens absolutely insures a thorough mixing of the oil with the sawdust and breaks up any lumps that might have been oil coated on the exterior and not oil coated on the interior of the lump. Asbes- 30 tos, preferably the long fiber, and of a type known commercially as #2 asbestos, is now mixed with the oiled sawdust in the proportion of one part of the finest oiled sawdust with one part of the coarser grade sawdust to 35 six (6) parts of the long fiber asbestos. These ingredients are carefully mixed in a suitable mixer or stirrer so that a complete homogeneous mass is obtained.

Other ingredients are now adapted to be 40 added to this mixture of two (2) parts of sawdust to six (6) parts of asbestos. To the foregoing mixture of asbestos and oiled sawdust is added thirty (30) parts of calcined magnesite ground to a grade of fineness 45 wherein substantially all of the said magnesite will pass through a screen having one hundred and twenty (120) meshes to the inch; plus eight (8) parts of crushed quartz of a type commercially known as mine run 50 and preferably comprising particles ranging in size from one-fourth ( $\frac{1}{4}$ ) to one-eighth ( $\frac{1}{8}$ ) of an inch; plus four (4) parts of white talc ground to comprise a fine powder; plus four (4) parts marble flour which is ground 55 very fine and comprises a very fine powder preferably of a grade known to the trade as #112; plus four (4) parts carborundum fire sand or a similar hard material. After all 60 of these materials have been obtained in substantially the proportions and of the characters specified they are thoroughly and completely mixed by suitable mixers and then subsequently packed for shipment. The material comprising the foregoing ingredients 65 may be suitably packed in bags, kegs, or bar-

rels, or other packages and transported to the place of use. In preparing this material for use a suitable binder is made up by dissolving magnesium chlorid in water until a solution is obtained which tests substantially 70 twenty - three (23) degrees on a Baumé heavy liquid hydrometer. The dry material comprising the ingredients above specified, in substantially the proportions set forth, is suitably mixed with the magnesium chlorid 75 binder to a consistency of mortar or paste and is then applied to form a roof or similar structure, and preferably is applied in thicknesses ranging from three-eighths ( $\frac{3}{8}$ ) of an inch to one-half ( $\frac{1}{2}$ ) of an inch over suitable 80 sheeting or supporting members and is surface-treated by floating and troweling, as is common in the art. When the liquid is mixed with the dry material a chemical reaction takes place and gases are emitted 85 thereby causing a temporary effervescence of the material together with a slight rise in temperature. The effervescence lasts but a short time and has usually disappeared by the time a workman can mix a suitable 90 amount and apply the same in place. In view of the fact that the liquid used has an extremely low freezing point ordinary winter weather does not interfere with the outside use of this material so that work may be 95 carried on in winter as well as in summer in connection with the use of this composition.

The mixture sets rather quickly, within fifteen to twenty minutes after mixing, depending upon temperature and liquidity of 100 the mixture, and possesses great adhesiveness, so much so that a roof may be laid directly against walls, chimneys, etc., and attached thereto by troweling, thereby eliminating flashings, etc. 105

After this composition of matter has been prepared and applied it forms a relatively smooth jointless sheet of very tough elastic and at the same time hard material capable of resisting both fire and water and substantially unaffected by heat or cold. At the same time, because of its strength it may be laid in relatively thin layers, consequently providing a protective covering without undue weight. These factors render this material particularly adaptable for roofing and similar purposes. 110

Realizing that it may be possible to use other materials possessing the desired chemical and physical characteristics and that it 115 may be possible to slightly vary the proportions herein specifically set forth, I desire that it be understood that the specific ingredients and specific proportions are the preferred materials and proportions so far as I 120 am at present aware.

Having described my invention, what I claim is:

1. A plastic composition adapted for use 130 in forming roofs and similar structures com-

- prising thirty (30) parts calcined magnesite; plus eight (8) parts crushed quartz; plus four (4) parts white talc; plus four (4) parts marble flour; plus four (4) parts carborundum fire sand; to which is added eight (8) parts of mixed long fiber asbestos and oiled sawdust mixed in proportion of one (1) part China wood oil to twenty (20) parts of sawdust and with two (2) parts of the oiled sawdust mixed with six (6) parts of long fiber asbestos.
2. A plastic composition adaptable for use in making roofs and similar structures, and comprising calcined magnesite; crushed quartz; white talc; marble flour; carborundum fire sand; and asbestos mixed with hard wood sawdust treated with China wood oil; substantially as specified.
3. A plastic composition adaptable to be used in making roofs and similar structures and comprising thirty (30) parts calcined magnesite; six (6) parts long fiber asbestos; two (2) parts sawdust treated with China wood oil; eight (8) parts crushed quartz; four (4) parts white talc; four (4) parts marble flour; four (4) parts carborundum fire sand; mixed with a binder comprising a solution of magnesia chlorid and water testing substantially twenty-three degrees Baumé; substantially as specified.
4. A plastic composition adapted to be used in forming roofs and the like, and comprising calcined magnesite; asbestos; sawdust treated with China wood oil; crushed quartz talc; marble flour; carborundum fire sand; mixed to a plastic state by adding a binder comprising magnesia chlorid dissolved in water, substantially as specified.
5. A plastic composition adapted for use in forming roofs and similar structures and comprising magnesia and silicon compounds mixed with asbestos and sawdust treated with China wood oil, substantially as specified.
6. A plastic composition adapted particularly to be used in forming roofs and similar
- structures, and comprising coarse quartz and fine calcined magnesite adapted to fill the voids between the coarser quartz, together with asbestos and hard wood sawdust 50 treated with China wood oil and mixed with magnesium chlorid in water, substantially as specified.
7. A plastic composition adapted for use in the making of roofs and similar structures and comprising quartz and of relatively large size, together with calcined magnesite adapted to fill the voids between the large size particles of quartz, and the water proofing material including China wood oil, 55 together with a long fiber material and treated with a magnesium chlorid binder adapted to cause certain of said materials to react chemically and form a composite mass of strong, hard, elastic qualities, substantially as specified.
8. A dry plastic composition adapted for use in making roofs and similar structures, comprising calcined magnesite; crushed quartz; white talc; marble flour; fire sand; 70 and asbestos mixed with a waterproofing carrier; substantially as specified.
9. A plastic composition adapted for use in making roofs and similar structures comprising calcined magnesite; crushed quartz; 75 white talc; marble flour; carborundum fire sand; and asbestos mixed with coarse and fine wood sawdust treated with China wood oil; substantially as specified.
10. A plastic composition adapted for use in making roofs and similar structures comprising thirty (30) parts of calcined magnesite; eight (8) parts of crushed quartz; four (4) parts of talc; four (4) parts of marble flour; four (4) parts of fire sand; and combined with a mixture comprising six (6) parts of asbestos with one part each of coarse and fine hard wood sawdust treated with China wood oil; substantially as specified.

WILHELM A. KOHNCKE.